

April 1, 1952

N. DRISCH ET AL

2,591,242

PROCESS FOR THE MANUFACTURE OF YARNS FROM  
HYDROXYLATED POLYVINYL COMPOUNDS  
Filed Jan. 19, 1950



INVENTORS  
Nicolas Drisch  
Paul Herrbach  
BY

*N. Drisch*  
Atty.

## UNITED STATES PATENT OFFICE

2,591,242

PROCESS FOR THE MANUFACTURE OF  
YARNS FROM HYDROXYLATED POLY-  
VINYLM COMPOUNDS

Nicolas Drisch and Paul Herrbach, Paris, France, assignors, by mesne assignments, to Textile and Chemical Research Company Limited, St. Peter Port, Guernsey, Channel Islands, a corporation of Great Britain

Application January 19, 1950, Serial No. 139,458  
In France February 1, 1949

5 Claims. (Cl. 18—54)

1

This invention relates to the manufacture of spun yarn from hydroxylated polyvinyl compounds in an ammonium sulphate spinning bath and has for an object to provide a novel and improved method for removing the ammonium sulphate from the yarn after spinning.

Other objects and advantages will be apparent as the nature of the invention is more fully disclosed.

The spinning of soluble rayon may be accomplished with the aid of various hydrophilic substances such as sodium alginate, carboxymethyl cellulose, etc.

Filaments obtained from sodium alginate solutions are lacking in elongation. They will not dissolve in aqueous medium, but only in slightly alkaline medium. Alginate threads are generally based on the calcium salt of alginic acid.

Filaments of the aluminum salt of cellulose-glycolic acid are not readily soluble in weak alkaline medium, but require more strongly alkaline media which may be harmful to the wool with which such products are often mixed.

The spinning of solutions of hydroxylated polyvinyl compounds is described in general in United States Patent No. 2,388,325. For example, aqueous solutions of polyvinyl alcohol are spun in a hot aqueous bath containing 35 per cent of ammonium sulphate. The filaments so obtained are stretched and collected in a spinning pot. The spinning is done with the usual equipment used for artificial textiles. The filaments obtained, impregnated with ammonium sulphate, are subjected to washing by a solution of 50 per cent acetone in water. This washing is tedious and difficult because of the low solubility of ammonium sulphate in the solvent mixture. Before drying, the cakes are re-treated with pure acetone.

Among the disadvantages of this process are the need for an organic solvent which must be recovered, the danger of explosion of the solvent-air mixture, and the solvent losses.

The present invention provides a simpler and more economical method of manufacturing yarn from hydroxylated polyvinyl compounds, such as polyvinyl alcohol.

According to the invention, the cakes of yarn are dried in a ventilated hot air drier, producing a package of yarn carrying ammonium sulphate in the form of an impalpably fine powder not affecting the strength of the individual filaments. The cake is re-wound by passing the yarn through a tensioning device set to introduce friction adapted to remove most of the ammonium sul-

2

phate powder coating the yarn. The yarn obtained is characterized by a very soft feel, complete independence of all filaments, and very satisfactory mechanical properties. The following example will afford a clearer understanding of the invention, but is of course in no way restrictive.

*Example*

10 A solution of 15 per cent polyvinyl alcohol of low viscosity is prepared by heating with water. This solution is readily filterable, even after cooling and has a viscosity of about 115 poises at 20° C. It is desirable to add 1 per cent of lauryl pyridinium chloride calculated on the polyvinyl alcohol. The resulting solution is filtered and deaerated.

15 The spinning is effected in a known way. The solution is spun in an aqueous bath containing 35 per cent ammonium sulphate at 50° C. from a spinneret having 30 holes of 10/100 mm. The thread is stretched 410 per cent between two rollers, the final speed being 40 to 55 min. The feed of the solution is controlled so as to yield 5 d. filaments. The resulting yarn is collected in cakes in a spinning pot with a speed of 6000 R. P. M. The resulting cakes are dried at 60° C. in a ventilated drier. They are unwound on ordinary spoolers, with the filament passing through a tensioning device set to produce tensions of the order of 1 gram per denier, e. g. in a grid tensioning device, to scrape off the adhering saline powder.

20 In the drawing the figure is a diagrammatic representation of one type of apparatus in which this process can be carried out.

25 Referring to the drawing the cake 10 of yarn 11 is unwound through guides 12 and 13 onto a spool 14 which is driven by a drive roller 15. Interposed between the guides 12 and 13 is a grid 30 tensioning and scraping device comprising sets of bars 16 and 17 which are interleaved and around which the yarn passes. The friction produced by the bars is controlled by varying the overlap of the two sets of bars. In operation the bars introduce sufficient friction to scrape the ammonium sulphate powder from the yarn as above described.

35 The resulting yarn has a dry strength of 1.90 grams per denier with an elongation at break of 40 per cent, and contains only a few per cent of salts, not enough to interfere with its use. It is very bright, flexible and soluble in water. It is suitable for all applications of soluble threads such as the manufacture of artificial embroidery or the like.

## What is claimed is:

1. The method of producing spun yarns from aqueous solutions of polyvinyl alcohol which comprises spinning said solution into a concentrated aqueous saline solution, stretching the spun filaments during the spinning operation, winding the yarn thus produced onto a package, drying the package to produce a yarn having adherent powder thereon, and rewinding the yarn from said package while passing the yarn with the adherent powder thereon over stationary friction members to scrape the adherent powder from the surface thereof.

2. The method of producing spun yarns from aqueous solutions of polyvinyl alcohol which comprises spinning said solution into a concentrated aqueous saline solution, stretching the spun filaments during the spinning operation, winding the yarn thus produced onto a package, drying the package to produce a yarn having adherent powder thereon, and rewinding the yarn from said package while passing the yarn with the adherent powder thereon over interleaved bars to apply friction to scrape the adherent powder from the surface thereof.

3. The method of producing spun yarns from aqueous solutions of polyvinyl alcohol which comprises spinning said solution into a concentrated aqueous saline solution, stretching the spun filaments during the spinning operation, winding the yarn thus produced onto a package, drying the package at a slightly elevated temperature with circulation of air thereover to produce a yarn having adherent powder thereon, and rewinding the yarn from said package while passing the yarn with the adherent powder thereon over stationary friction members to scrape the adherent powder from the surface thereof.

4. The method of producing spun yarns from aqueous solutions of polyvinyl alcohol which comprises spinning said solution into a concentrated aqueous solution of ammonium sulphate, stretching the spun filaments during the spinning operation, winding the yarn thus produced onto a package, drying the package to provide a yarn having ammonium sulphate powder adhering thereto, and rewinding the yarn from said package while passing the yarn with the adherent powder thereon over stationary friction members to scrape the adherent powder from the surface thereof.

5. The method of producing spun yarns from aqueous solutions of polyvinyl alcohol which comprises spinning said solution into a concentrated aqueous saline solution, stretching the spun filaments during the spinning operation, winding the yarn thus produced onto a package, 20 drying the package to produce a yarn having adherent powder thereon, and rewinding the yarn from said package while applying a stretching tension of approximately 1 gram per denier and scraping adherent powder from the surface thereof.

NICOLAS DRISCH.  
PAUL HERRBACH.

## REFERENCES CITED

30. The following references are of record in the file of this patent:

## UNITED STATES PATENTS

| Number       | Name          | Date           |
|--------------|---------------|----------------|
| 35 2,257,382 | Javery et al. | Sept. 30, 1941 |
| 2,388,325    | Houtz         | Nov. 6, 1945   |